# EUROPEAN PATENT SPECIFICATION

(11) **EP 0 055 272 B1**
(45) Date of publication and mention of the grant of the patent: **27.11.1985**
(21) Application number: 81901799.7
(22) Date of filing: 02.07.1981
(51) Int. Cl.: C25D 15/02

(54) **COMPOSITE ELECTRODEPOSITED COATING AND METHOD OF FORMING THE SAME**
ELEKTROLYTISCH AUFGEBRACHTER VERBUNDÜBERZUG UND VERFAHREN ZU SEINER HERSTELLUNG
REVETEMENT COMPOSITE ELECTRO-DEPOSE ET PROCEDE DE FORMATION DE CELUI-CI

(30) Priority: 02.07.1980 GB 8021614
(43) Date of publication of application: 07.07.1982
(73) Proprietor: BAJ Limited, Weston-Super-Mare Avon BS24 8PD (GB)
(72) Inventor: KEDWARD, Eric Charles, Avon (GB); ADDISON, Colin Anthony, Hutton Weston-Super-Mare (GB); Honey, Francis John, Burnham-On-Sea Somerset (GB)
(74) Representative: Rees, David Christopher
(86) International application number: GB8100124
(87) International publication number: WO8200162

## Description

The present invention relates to a composite electrodeposited coating comprising a metal matrix electrodeposited from a plating bath, the matrix incorporating particles deposited simultaneously from the bath in which the particles are substantially insoluble.

It has been proposed to employ various metals as the matrix, for example nickel and cobalt, and it has been proposed to employ various particles, for example silicon carbide, chromium carbide and graphite.

It is an object of the present invention to provide a coating which is highly resistant to oxidation and/or to corrosion, for example in a sulphur-containing environment, at high temperatures. Such conditions might occur in jet or rocket engines.

It is a further object of the invention to provide a resistant coating which remains substantially unaffected by thermal cycling.

US 3057048 (Hirakis) describes a method of protecting niobium in a high temperature oxidising environment by electro-depositing a coating comprising a matrix of iron chromium nickel or cobalt incorporating various solid particles for example alumina, thoria, silicon, aluminium, chromium and boron. The coating is found to have a particulate content of from 5 to 20% by volume.

It is a further object of the invention to provide a resistant coating which has a high particulate content and which is not prone to spallation.

According to one aspect of the invention, a composite electrodeposited coating is characterised in that the particles comprise a combination of particles of or containing chromium, particles of or containing aluminium and particles of an oxide of a rare earth metal and/or an oxide of zirconium, titanium or hafnium.

The particles other than the oxide particles may comprise pure chromium powder and pure aluminium powder, or an alloy of chromium and aluminium in powder form, or an alloy of chromium and aluminium in powder form mixed with either both or one of pure aluminium or chromium, or one further possibility is to have a small quantity of a rare earth metal or a Group IV metal alloyed with either chromium or aluminium or both.

Preferably the metal matrix comprises nickel or cobalt and the coating may be used to coat any suitable substrate for example steel, high temperature creep-resistant nickel alloys, nonferrous and light alloys and non-metallic substances with an outer conductive layer.

The oxide present in the coating preferably comprises "lime-stabilized" zirconia. The oxide may constitute from 0.01 to 5% of the coating, preferably about 2% by weight, and may be present in the size range up to 10 pm.

The chromium present in the coating may comprise up to 40% by weight of the coating, preferably comprising 10 to 20%, for example 15%. The aluminium present in the coating may comprise up to 25% by weight of the coating and preferably comprises 10 to 20%.

The particles may be up to 10 pm in diameter and preferably fall largely within the range of 1 to 2 um.

According to another aspect of the present invention a method of forming a composite coating is characterised in that the particles comprise a combination of particles of or containing chromium, particles of or containing aluminium, and particles of an oxide of a rare earth metal and/or an oxide of zirconium, titanium or hafnium.

After deposition the coating may be further heat treated, either in use or for example by being held at 1000°C for 4 hours.

It has been found that a layer of aluminium oxide forms over the surface of the coating by aluminium atoms diffusing to the surface and oxidising. This process carries on until the surface is covered. After the initial oxide layer has covered the surface, it is believed that further oxide can only form by either the aluminium diffusing through the oxide to react with further oxygen at the surface, or oxygen diffusing through the oxide to react with aluminium to form more oxide at the metal oxide interface. One further possibility may be that both mechanisms are operating and fresh oxide is also formed within that already existing.

In general, if a metal atom diffuses outwards through the oxide it may leave behind a vacancy. In the case of known castings it is believed that during the course of time the vacancies would normally coalesce at the interface between the metal and oxide to form voids such that the oxide would only be attached to the parent metal at a few places. Furthermore, the oxide formed might have a greater volume than the original metal from which it has been formed and so a compressive stress would develop in the growing oxide layer. This might give rise to a complicated stress situation at the oxide-metal interface which is believed to consist mainly of shear stresses and also transverse stress acting to pull the oxide away from the metal. The net result of these stresses coupled with the lack of coherency at the interface would be that the oxide would spall off and expose fresh metal to the hot gas. This process would repeat itself and so the metal would be progressively lost.

A problem which may arise if oxide spallation does not occur is that the oxide simply gets thicker as time goes on and the component gets weaker as the cross section of the metal decreases.

One method by which these problems may be overcome is to reduce simultaneously the rates at which the oxygen and metal diffuse through the oxide and to provide a means by which the vacancies may be annihilated and so prevent void formation. It is in this way that the inclusion of the oxide particles, which are both thermodynamically stable and chemically stable in an oxidising atmosphere, may greatly improve the adhesion of the aluminium oxide to the matrix metal at the surface of the coating. It is believed that the effect is achieved in three ways, either singly or in combination.

The first of these is the "stress relief" mechanism in which the presence of oxide particles at the coating's surface provides "dead spots" over which the developing oxide film can grow laterally thereby relieving any stresses in the film. The second is the "vacancy sink" mechanism in which the vacancies left by aluminium atoms diffusing to the surface to react with oxygen are at least partially filled by oxide molecules so that the oxide particles undergo a rearrangement to occupy the voids which effectively "diffuse" through the matrix. The third is simply a reduction in the diffusion coefficients through the growing surface oxide layer of either the metal ions or the oxygen atoms or both.

The above enhancement in adhesion is described with reference to aluminium and its oxide; however it is to be understood that the description is also applicable to chromium and its oxide, and therefore also to aluminium/chromium alloy and both oxides. It has been found in practice that an increase in the relative amount of aluminium results in a predominance of aluminium oxide in the outer layers of the coating which is then more resistant in an oxidising environment while an increase in the relative amount of chromium results in a predominance of chromium oxide which is more resistant to a sulphur-containing environment. Thus, by adjusting the relative quantities of aluminium and chromium the usability of the coating can be varied.

According to a further aspect of the invention, a method of forming a composite coating is characterised in that the particles comprise a combination of particles of or containing chromium and particles of an oxide of a rear earth metal and/or oxide of zirconium titanium or hafnium, and by subsequently aluminising the coating.

Preferably, the particles also include an aluminium-containing substance and, preferably, the aluminising step comprises a pack-aluminising process. In this process the material used may be aluminium powder, or a mixture of aluminium and aluminium oxide. Preferably, the aluminium is in the form of an alloy with chromium.

The pack-aluminising is carried out at a high temperature. The aluminium is believed to diffuse into the surface of the electrodeposited coating and thus form a bond. The coating may be subsequently heat treated, for example by being held at 1000°C for about 4 hours, or may be heat treated in use.

The substances described with reference to the first method may also be used in the second method with the same effect.

The coating process may involve an electrolytic or an electroless method and may be carried out using the apparatus and operating conditions described in the Applicants' British Patents Nos. 1 218 179, 1 224 166, 1 329 081 and 1 347 184.

One specific example of a process applying a coated in accordance with the invention will now be described.

### Example 1

Using the apparatus described in our copending British Patent Application No. 7906521, Serial No. a stainless steel panel two inches (50.8 mm) by one inch (25.4 mm) by one-eighth of an inch (3.2 mm) thick was provided with a composite coating comprising a cobalt matrix including particles of lime-stabilised zirconia and particles of aluminium/chromium alloy. The tank was filled with a solution comprising 450 grams per litre of cobalt sulphate, 30 grams per litre of boric acid and 2.5 grams per litre of sodium chloride. To 125 litres of this solution contained in the tank was added 10 millilitres of Canning's anti-pit liquid.

The panel to be coated was given a pretreatment comprising immersion in a cyanide cleaner for two minutes followed by a water rinse etching by immersion for 30 seconds in a 50% sulphuric acid followed by a water rinse, and a nickel strike by plating in a nickel bath for three minutes at a current density of 3.9 amps per square decimetre. The panel was secured in a plating barrel and connected to a cathode contact. 40 grams per litre of barrel capacity of lime-stabilised zirconia powder and 600 grams per litre of barrel capacity of chromium/aluminium alloy powder, both with a mean particle size of to 5 pm, were added to the barrel and the opening in the barrel through which the panel to be coated and the powder were admitted was closed. The barrel was then completely submerged in the solution in the tank and was rotated at three revolutions per minute while composite plating took place at a voltage of between 2.5 and 3 volts with a current density of approximately 2.7 amps per square decimetre. The solution temperature was maintained at 50°C and the solution had a pH of between 4.5 and 5. After plating has proceeded for a time sufficient to give a thickness of plating of 0.05 mm, plating was stopped. The panel was then held at 1000°C for 4 hours, cooled and examined. It was found that the panel had been given a tenacious coating having an even distribution of particles. The coating had a particle content of approximately 2% by volume of zirconia and 30% by volume of chromium/ aluminium alloy.

## Claims

1. A composite electrodeposited coating comprising a metal matrix electrodeposited from a plating bath, the matrix incorporating particles deposited simultaneously from the bath in which the particles are substantially insoluble charac- teristised in that the particles comprise a combination of particles of or containing chromium particles of or containing aluminium, and particles of an oxide of a rare earth metal and/or an oxide of zirconium, titanium or hafnium.

2. A coating as claimed in Claim 1 characterised in that the matrix metal is nickel or cobalt.

3. A coating as claimed in Claim 1 or Claim 2 characterised in that the oxide is "lime-stabilised" zirconia.

4. A coating as claimed in any preceding claim characterised in that the particles further include particles of aluminium oxide.

5. A coating as claimed in any preceding claim characterised in that the particles are up to 10 11m in diameter.

6. A coating as claimed in any preceding claim characterised in that the aluminium present comprises up to 25% by weight of the coating.

7. A coating as claimed in any preceding claim characterised in that the chromium present comprises up to 40% by weight of the coating.

8. A coating as claimed in any preceding claim characterised in that the particles of aluminium comprise pure aluminium powder.

9. A coating as claimed in any preceding claim characterised in that the particles of chromium comprise pure chromium powder.

10. A coating as claimed in any of Claims 1 to 6 characterised in that the particles containing chromium and the particles containing aluminium comprise an alloy of aluminium and chromium in powder form.

11. A method of forming a composite coating comprising electrodepositing a metal matrix from a plating bath and simultaneously depositing particles which are substantially insoluble in the plating bath, characterised in that the particles comprise a combination of particles of or containing chromium, particles of or containing aluminium, and particles of an oxide of a rare earth metal and/or an oxide of zirconium titanium or hafnium.

12. A method of forming a composite coating comprising electrodepositing a metal matrix from a plating bath and simultaneously depositing particles which are substantially insoluble in the plating bath characterised in that the particles comprise a combination of particles of or containing chromium and particles of an oxide of a rare earth metal and/or oxide of zirconium, titanium or hafnium, and by subsequently aluminising the coating.

13. A method as claimed in Claim 12 characterised in that the particles further include an aluminium-containing substance.

14. A method as claimed in Claim 12 characterised in that the coating is pack aluminised.

15. A method as claimed in any of Claims 11 to 14 characterised in that the matrix metal is nickel or cobalt.

16. A method as claimed in any of Claims 11 to 15 characterised in that the oxide is "lime-stabilised" zirconia.

17. A method as claimed in any of Claims 11 to 16 characterised in that the particles further include particles of aluminium oxide.

18. A method as claimed in any of Claims 11 to 17 characterised in that the particles are up to 10 pm in diameter.

19. A method as claimed in any of Claims 11 to 18 characterised in that the aluminium-containing substance comprises pure aluminium powder.

20. A method as claimed in any of Claims 11 to 19 characterised in that the particles of chromium comprise pure chromium powder.

21. A method as claimed in any of Claims 11 to 18 characterised in that the particles containing chromium and the particles containing aluminium comprise an alloy of aluminium and chromium in powder form.

## Patentansprüche

1. Ein elektrolytisch aufgebrachter Verbundüberzug, bestehend aus einem aus einem Plattierungsbad elektrolytisch aufgebrachten metallischen Grundgefüge, wobei das Grundgefüge Teilchen umfaßt, die gleichzeitig aus dem Bad abgeschieden wurden, in dem die Teilchen im wesentlichen unlöslich sind, dadurch gekennzeichnet, daß die Teilchen eine Kombination aus Chromteilchen oder Chrom enthaltenden Teilchen aus Aluminiumteilchen oder Aluminium enthaltenden Teilchen und aus Teilchen eines Oxids eines seltenen Erdmetalls und/oder eines Zirkonium-, Titan- oder Hafniumoxids sind.

2. Ein Überzug wie in Anspruch 1, dadurch gekennzeichnet, daß das Metall des Grundgefüges Nickel oder Kobalt ist.

3. Ein Überzug wie in Anspruch 1 oder Anspruch 2, dadurch gekennzeichnet, daß das Oxid "kalk-stabilisierte" Zirkonerde ist.

4. Ein Überzug wie in einem der vorhergehenden Ansprüche, dadurch gekennzeichnet, daß die Teilchen des weiteren Aluminiumoxidteilchen umfassen.

5. Ein Überzug wie in einem der vorhergehenden Ansprüche, dadurch gekennzeichnet, daß die Teilchen einen Durchmesser von bis zu 10 11m haben.

6. Ein Überzug wie in einem der vorhergehenden Ansprüche, dadurch gekennzeichnet, daß das vorhandene Aluminium bis zu 25 Gew.-% des Überzugs beträgt.

7. Ein Überzug wie in einem der vorhergehenden Ansprüche, dadurch gekennzeichnet, daß das vorhandene Chrom bis zu 40 Gew-% des Überzugs beträgt.

8. Ein Überzug wie in einem der vorhergehenden Ansprüche, dadurch gekennzeichnet, daß die Aluminiumteilchen aus reinem Aluminiumpulver bestehen.

9. Ein Überzug wie in einem der vorhergehenden Ansprüche, dadurch gekennzeichnet, daß die Chromteilchen aus reinem Chrompulver bestehen.

10. Ein Überzug wie in einem der Ansprüche 1 bis 6, dadurch gekennzeichnet, daß die Chrom enthaltenden und die Aluminium enthaltenden Teilchen aus einer Legierung aus Aluminium und Chrom in Pulverform bestehen.

11. Ein Verfahren zur Herstellung eines Verbundüberzuges, umfassend das elektrolytische Aufbringen eines metallischen Grundgefüges aus einem Plattierungsbad und die gleichzeitige Abscheidung von Teilchen, die in dem Plattierungsbad im wesentlichen unlöslich sind, dadurch gekennzeichnet, daß die Teilchen eine aus Chromteilchen bestehende oder aus Aluminium bestehende oder Aluminium enthaltende, und aus Teilchen eines Oxids eines seltenen Erdmetalls und/oder eine Zirkonium-, Titan- oder Hafniumoxids bestehende Kombination.

12. Ein Verfahren zur Herstellung eines Verbundüberzuges durch galvanische Fällung einer Metallmatrize aus einem Galvanisierbad und gleichzeitige Abscheidung von Teilchen, die in dem Galvanisierbad im wesentlichen unlöslich sind, dadurch gekennzeichnet, daß die Teilchen eine Kombination aus Chromteilchen oder Chrom enthaltenden Teilchen, und aus Teilchen eines Oxids eines seltenen Erdmetalls und/oder eines Zirkonium-, Titan- oder Hafniumoxids sind, und durch anschließende Veraluminierung des Überzuges.

13. Ein Verfahren wie in Anspruch 12, dadurch gekennzeichnet, daß die Teilchen des weiteren eine aluminiumhaltige Substanz enthalten.

14. Ein Verfahren wie in Anspruch 12, dadurch gekennzeichnet, daß der Überzug im Umpackungsverfahren veraluminiert wird.

15. Ein Verfahren wie in einem der Ansprüche 11 bis 14, dadurch gekennzeichnet, daß das Metall des Grundgefüges Nickel oder Kobalt ist.

16. Ein Verfahren, wie in einem der Ansprüche 11 bis 15, dadurch gekennzeichnet, daß das Oxid "kalk-stabilisierte" Zirkonerde ist.

17. Ein Verfahren wie in einem der Ansprüche 11 bis 16, dadurch gekennzeichnet, daß die Teilchen des weiteren Aluminiumoxidteilchen umfassen.

18. Ein Verfahren wie in einem der Ansprüche 11 bis 17, dadurch gekennzeichnet, daß die Teilchen einen Durchmesser von bis zu 10 pm haben.

19. Ein Verfahren wie in einem der Ansprüche 11 bis 18, dadurch gekennzeichnet, daß die aluminiumhaltige Substanz aus reinem Aluminiumpulver besteht.

20. Ein Verfahren wie in einem der Ansprüche 11 bis 19, dadurch gekennzeichnet, daß die Chromteilchen aus reinem Chrompulver bestehen.

21. Ein Verfahren wie in einem der Ansprüche 11 bis 18, dadurch gekennzeichnet, daß die chromhaltigen und aluminium-haltigen Teilchen aus einer Legierung aus Aluminium und Chrom in Pulverform bestehen.

## Revendications

1. Un revêtement composite déposé électrolytiquement comprenant une matrice métallique déposée électrolytiquement à partir d'un bain de plaquage, la matrice comportant des particules déposées simultanément à partir du bain dans lequel les particules sont sensiblement insolubles, caractérisé en ce que les particules comprennent une combinaison de particules de ou contenant du chrome, de particules de ou contenant de l'aluminium et de particules d'un oxyde d'un métal de terre rare et/ou d'un oxyde de zirconium, de titane ou d'hafnium.

2. Un revêtement tel que revendiqué dans la revendication 1, caractérisé en ce que le métal de matrice est du nickel ou du cobalt.

3. Un revêtement tel que revendiqué dans la revendication 1 ou la revendication 2, caractérisé en ce que l'oxyde est de l'oxyde de zirconium "stabilisé à la chaux".

4. Un revêtement tel que revendiqué dans une quelconque des revendications précédentes, caractérisé en ce que les particules comprennent en outre des particules d'oxyde d'aluminium.

5. Un revêtement tel que revendiqué dans une quelconque des revendications précédentes, caractérisé en ce que les particules ont un diamètre jusqu'à 10 microns.

6. Un revêtement tel que revendiqué dans une quelconque des revendications précédentes, caractérisé en ce que l'aluminium présent forme jusqu'à 25% en poids du revêtement.

7. Un revêtement tel que revendiqué dans une quelconque des revendications précédentes, caractérisé en ce que le chrome présent forme jusqu'à 40% en poids du revêtement.

8. Un revêtement tel que revendiqué dans une quelconque des revendications précédentes, caractérisé en ce que les particules d'aluminium comprennent de la poudre d'aluminium pur.

9. Un revêtement tel que revendiqué dans une quelconque des revendications 'précédentes, caractérisé en ce que les particules de chrome comprennent de la poudre de chrome pur.

10. Un revêtement tel que revendiqué dans une quelconque des revendications 1 à 6, caractérisé en ce que les particules contenant du chrome et les particules contenant de l'aluminium comprennent un alliage d'aluminium et de chrome sous forme de poudre.

11. Un procédé de formation d'un revêtement composité, consistant à déposer électrolytiquement une matrice métallique à partir d'un bain de plaquage et à déposer simultanément des particules qui sont sensiblement insolubles dans le bain de plaquage, caractérisé en ce que les particules comprennent une combinaison de particules de ou contenant du chrome, de particules de ou contenant de l'aluminium et de particules d'un oxyde d'un métal de terre rare et/ou d'un oxyde de zirconium, de titane ou d'hafnium.

12. Un procédé de formation d'un revêtement composite, consistant à déposer électrolytiquement une matrice métallique à partir d'un bain de plaquage et à déposer simultanément des particules qui sont sensiblement insolubles dans le bain de plaquage, caractérisé en ce que les particules comprennent une combinaison de particules de ou contenant particules d'un oxyde d'un métal de terre rare et/ou d'un oxyde de zirconium, de titane ou d'hafnium, et à aluminiser ultérieurement le revêtement.

13. Un procédé tel que revendiqué dans la revendication 12, caractérisé en ce que les particules comprennent en outre une substance contenant de l'aluminium.

14. Un procédé tel que revendiqué dans la revendication 12, caractérisé en ce que le revêtement est aluminisé.

15. Un procédé tel que revendiqué dans une quelconque des revendications 11 à 14, caractérisé en ce que le métal de matrice est du nickel ou du cobalt.

16. Un procédé tel que revendiqué dans une quelconque des revendications 11 à 15, caractérisé en ce que l'oxyde est de l'oxyde de zirconium "stabilisé à la chaux".

17. Un procédé tel que revendiqué dans une quelconque des revendications 11 à 16, caractérisé en ce ce que les particules comprennent en outre des particules d'oxyde d'aluminium.

18. Un procédé tel que revendique dans une quelconque des revendications 11 à 17, caractérisé en ce que les particules ont un diamètre jusqu'à 10 microns.

19. Un procédé tel que revendiqué dans une quelconque des revendications 11 à 18, caractérisé en ce que la substance contenant de l'aluminium comprend une poudre d'aluminium pur.

20. Un procédé tel que revendiqué dans une quelconque des revendications 11 à 19, caractérisé en ce que les particules de chrome comprennent de la poudre de chrome pur.

21. Un procédé tel que revendiqué dans une quelconque des revendications 11 à 18, caractérisé en ce que les particules contenant du chrome et les particules contenant de l'aluminium comprennent un alliage d'aluminium et de chrome sous forme de poudre.
